

# United States Patent

[11] 3,620,937

[72] Inventors **John A. Lisowski;**  
**Frank B. Lisowski, both of Newport, Mich.**  
[21] Appl. No. **849,157**  
[22] Filed **Aug. 11, 1969**  
[45] Patented **Nov. 16, 1971**  
[73] Assignee **Natural Products Company**  
**Newport, Mich.**

[54] **METHOD AND ELECTROLYTE FOR  
ELECTROPLATING BRASS**  
**6 Claims, No Drawings**

[52] U.S. Cl. .... **204/44,**  
**204/DIG. 2**  
[51] Int. Cl. .... **C23b 5/36,**  
**C23b 5/46**

[50] **Field of Search** ..... **204/44,**  
**123; 106/1; 117/130 E**

[56] **References Cited**  
**UNITED STATES PATENTS**  
**3,440,152 4/1969 Lisowski et al. .... 204/44**  
**Primary Examiner—G. L. Kaplan**  
**Attorney—Whittemore, Hulbert & Belknap**

**ABSTRACT:** An electrolyte and process for electrodeposition of brass from an aqueous alkaline cyanide bath containing zinc cyanide, copper cyanide and an additive of cyclohexanone resulting in a uniform color of deposit and elimination of streaks and nonuniformity in color.

**METHOD AND ELECTROLYTE FOR ELECTROPLATING  
BRASS**

**BACKGROUND OF THE INVENTION**

The invention relates to the electrodeposition of brass and more particularly to brass alloy plating solutions which deposit a high-zinc alloy. It has been found that under certain conditions the electroplated surfaces have areas of different color with lines of demarcation which cannot be eliminated by subsequent metal depositions.

This is particularly true in alkaline high-zinc brass alloy plating solutions having metal ratios of 30 to 45 percent copper and 70 to 55 percent zinc. Under certain conditions of cyanide and caustic concentrations, or under certain conditions of contamination, the deposited brass alloys have different compositions on surfaces having nonuniform current densities. Usually, the zinc-rich deposit will be found in the low-current density area. This, at times, will create surfaces of different color, with the alloy highest in zinc being a silver color, while the alloy with the lower concentration remaining pink or yellow, and the interface having lines of demarcation which often cannot be erased by subsequent metal depositions.

We have discovered a remedy which overcomes the above-mentioned nonuniformity of the brass deposits and tends to promote more uniform deposits free from discoloration and staining.

Our invention comprises an additive for brass-plating solutions consisting of cyclohexanone. When cyclohexanone is used in concentrations of 2.3 fluid ounces (80-90 ml.) per thousand gallons of plating solution up to the limit of solubility of cyclohexanone in that solution, a more uniform deposition is obtained over a wide current density range. This results in a uniform color of deposit over the entire surface of the plated article.

A typical high-zinc brass plating bath has the following analysis:

|                       | Ounces per Gallon |
|-----------------------|-------------------|
| Sodium cyanide (free) | 8.00              |
| Sodium hydroxide      | 5.00              |
| Copper cyanide        | 2.57              |
| Copper as metal       | 1.80              |
| Zinc cyanide          | 5.53              |
| Zinc metal            | 3.10              |
| Cyclohexanone         | 0.002             |
| Ratio: copper to zinc | 36.8 to 63.2      |

The above brass-plating bath can be used with conventional brass anodes containing zinc in the range of 55 percent to 60 percent and copper in the range of 40 to 45 percent and an electrical current density of 30 to 40 amperes per square foot.

In its broader aspects, the invention may be carried out with the ingredients in the following wider ranges:

|                       | Ounces per gallon            |
|-----------------------|------------------------------|
| Sodium cyanide (free) | 6.50 to 9.00                 |
| Sodium hydroxide      | 2.50 to 6.00                 |
| Copper cyanide        | 1.41 to 4.23                 |
| Copper as metal       | 1.00 to 3.00                 |
| Zinc cyanide          | 2.60 to 6.82                 |
| Zinc metal            | 1.45 to 3.80                 |
| Total zinc and copper | 3.30 to 5.40                 |
| Cyclohexanone         | 0.002 to limit of solubility |
| Ratio: Cu/Zn          | 30/70 to 55/45               |

In practicing the invention, the cyclohexanone may be added to the plating solution in any convenient way to produce a true solution. Since cyclohexanone has limited solubility in water and lower solubility in aqueous solutions having high concentrations of electrolytes, direct addition of cyclohexanone to brass-plating solution forms little droplets over the surface which dissolve slowly. Therefore, work to be plated should not be introduced into the bath until the additive has had an opportunity to dissolve as otherwise there can be skips in plating on the surface of the parts being immersed for plating. In order to obtain more rapid solution of cyclohex-

anone, in the plating bath, it is desirable to first dissolve the cyclohexanone in solvents which are mutually soluble in cyclohexanone and the plating solution. Examples of such solvents are formaldehyde, acetone, alcohols, diethylene glycol methyl ether, etc. These tend to disperse the cyclohexanone for a larger contact with the solution.

If proprietary dry powder additives are regularly used to give a plating bath certain desirable properties, cyclohexanone can be blended with these additives and introduced into the plating bath. This method will likewise disperse the cyclohexanone for a more rapid solution.

The use of cyclohexanone in commercial brass plating depends somewhat upon the nature of the plating operations. If the conditions are such that uniform color quality is being obtained, then the addition of cyclohexanone is unnecessary until such time as trouble appears. In general, it may be stated that the present invention is useful under two different types of conditions. First, when the plating bath is relatively free from contaminants and, second, when the plating operations require the use of special additives as brighteners or for other purposes. Such additives sometimes hasten the deterioration of color uniformity and would therefore tend to make the plated articles of inferior quality. When this occurs, it can be remedied by adding cyclohexanone in accordance with this invention. The present invention is of great value when indium is added to brass-plating baths as disclosed in U.S. Pat. No. 3,440,152, dated Apr. 22, 1969. Indium acts like a contaminant, but any detrimental effect on color uniformity can be remedied by using cyclohexanone as set forth herein.

What we claim as our invention is:

1. A bath for electrodeposition of brass comprising an aqueous alkaline solution of soluble compounds within the following ranges:

|                       | Ounces per gallon            |
|-----------------------|------------------------------|
| Sodium cyanide (free) | 6.50 to 9.00                 |
| Sodium hydroxide      | 2.50 to 6.00                 |
| Copper cyanide        | 1.41 to 4.23                 |
| Copper as metal       | 1.00 to 3.00                 |
| Zinc cyanide          | 2.60 to 6.82                 |
| Zinc metal            | 1.45 to 3.80                 |
| Total zinc and copper | 3.30 to 5.40                 |
| Cyclohexanone         | 0.002 to limit of solubility |
| Ratio: Cu/Zn          | 30/70 to 55/45               |

2. A bath according to claim 1 in which the compounds are present in approximately the following amounts:

|                       | Ounces per Gallon |
|-----------------------|-------------------|
| Sodium cyanide (free) | 8.00              |
| Sodium hydroxide      | 5.00              |
| Copper cyanide        | 2.57              |
| Copper as metal       | 1.80              |
| Zinc cyanide          | 5.53              |
| Zinc metal            | 3.10              |
| Cyclohexanone         | 0.002             |
| Ratio: copper to zinc | 36.8 to 63.2      |

3. In the process of electroplating brass from an aqueous alkaline cyanide bath comprising zinc and copper in solution, the improvement in said process of having cyclohexanone present in solution in an amount sufficient to prevent nonuniformity of deposits on surfaces having nonuniform current densities.

4. A process according to claim 3 in which cyclohexanone is present in a concentration at least 2 ounces per 1,000 gallons of solution.

5. A process according to claim 3 in which the plating bath is within the following ranges:

|                       | Ounces per gallon |
|-----------------------|-------------------|
| Sodium cyanide (free) | 6.50 to 9.00      |
| Sodium hydroxide      | 2.50 to 6.00      |
| Copper cyanide        | 1.41 to 4.23      |
| Copper as metal       | 1.00 to 3.00      |
| Zinc cyanide          | 2.60 to 6.82      |
| Zinc metal            | 1.45 to 3.80      |
| Total zinc and copper | 3.30 to 5.40      |

Cyclohexanone

Ratio: Cu/Zn

0.002 to limit  
of solubility  
30/70 to 55/45Sodium cyanide (free)  
Sodium hydroxide  
Copper cyanide  
Copper as metal  
Zinc cyanide  
Zinc metal  
Cyclohexanone  
Ratio: copper to zinc8.00  
5.00  
2.57  
1.80  
5.53  
3.10  
0.002  
to 63.2

6. A process according to claim 3 in which the plating bath  
has approximately the following composition:

Ounces per gallon

\* \* \* \* \*

10

15

20

25

30

35

40

45

50

55

60

65

70

75